

Feb. 11, 1930.

R. J. NORTON

1,746,493

BRAKE DRUM

Filed Feb. 2, 1929



Inventor

RAYMOND J. NORTON

By M. W. Melonkey, Jewmer & Jewmer  
Attorneys

## UNITED STATES PATENT OFFICE

RAYMOND J. NORTON, OF WASHINGTON, DISTRICT OF COLUMBIA

## BRAKE DRUM

Application filed February 2, 1929. Serial No. 337,022.

This invention relates to improvements in selected portion of the brake drum may be  
brake drums. treated in a very simple and economical manner to change the physical properties of that

Heretofore, brake drums have been made of either cast iron or low carbon deep-draw 5 steel. These metals, as is known, are relatively easily corroded. As a result of this corrosion, the drum not only becomes unsightly, but is also seriously weakened, due to the oxidation of the iron structure. In 10 brake drums, oxidation is greatly accelerated due to the catalytic effect of the generated heat of friction.

Prior to this time, relatively little attention has been paid to the problem of increasing 15 the efficiency and life of brake drums by rendering them relatively non-corrodible. The oxidation of the drum may obtain not only on the exterior surface, which is exposed to moisture, but may also take place 20 on the interior of the braking flange. The possibility of corrosion of the braking flange will be more readily appreciated when it is considered that, in certain types of lining, 25 materials are employed which are corrosive in action. For example, if the brake band had incorporated in it an appreciable amount of a corrosive substance, such for example as sodium chloride, there would be a decided 30 tendency to corrosion.

The major object of this invention is to provide a brake drum of which the frictional surface is comprised of a metallic substance of relatively low corrodibility.

Another object is to provide a brake structure both the interior and exterior surfaces of which may be economically treated to 35 lower the corrodibility.

The invention is illustrated diagrammatically in the single figure of the drawing.

In the prior application Serial No. 274,675, filed May 2, 1928, there was described a process by which a ferruginous brake drum might be cheaply treated to provide an exposed surface having an increased resistance to corrosion over that obtaining for ordinary iron.

The present invention is concerned with this same general problem, but the increased resistance to corrosion is secured by a different method.

According to the present invention, any

selected portion of the brake drum may be treated in a very simple and economical manner to change the physical properties of that portion, among which is an increased resistance to corrosion. The invention comprises 55 the concept of treating the drum so as to form as a constituent part of the ferruginous material a coating or molecularly bonded skin of a ferroso-ferric phosphate.

The invention may be effectuated by parkerizing any desired portion of the drum. The parkerizing process seems to be based on the fact that phosphoric acid will react with iron to precipitate a ferrous phosphate 60 on a metal surface. The compound which 65 is formed as a result of the process appears to be a basic ferroso-ferric phosphate and its action is to greatly increase the resistance to ordinary oxidation.

The particular manner of treating the 70 drum may be widely varied. As an example, the pre-formed drum may first be cleaned by immersion in a suitable caustic soda solution, maintained at a temperature of 200° F. 75 more or less. After cleaning in the caustic, the drum is removed and washed with hot water and then is subjected to a pickling in a five-percent sulphuric acid pickle. The pickle bath preferably contains a small 80 amount of sodium bi-sulphate. As is known, the composition of the bath is such that sulphur di-oxide is liberated and is free to act 85 upon the work. The sulphur di-oxide apparently is generated to reduce some of the difficultly soluble higher oxides of iron to lower oxides.

After the pickling operation, the drum may then be immersed in the parkerizing solution. The deposit of the desired phosphatic salt may be localized to any area by covering 90 the portions which are not treated with a suitable protective coating.

The treating solution may be made up by treating iron filings with concentrated phosphoric acid to prepare a paste of ferrous phosphate. This paste may then be added to a weak solution of boiling phosphoric acid, in which is incorporated a suitable amount of an oxidizing agent such as manganese di-oxide. 95 The drum may be maintained in the heated 100

bath for, say, from one to three hours, depending on the degree of protection desired. When the processing is completed, the drum may be removed and dried, and then dipped in a suitable oleaginous mixture.

It will be understood that there exists a wide range of choice in the particular processing solution which is employed. For example, the drum may be treated with a solution made up of phosphoric acid, sodium dichromate and water or, if desired, the drum may be subjected to the action of a mist of phosphorus pentoxide in water vapor. Any such similar treatment which will form a molecular skin or coating on the drum which comprises a compound having the protective features of a basic ferroso-ferric phosphate may be employed.

As will be understood, the particular character of the coating may be somewhat varied by varying the initial cleaning treatment. The character of the final coat will change somewhat, depending upon whether the preliminary cleaning of the metal has been by sand blast, rubbing or pickling.

This method of treatment presents many advantages. The process, as such, is a very economical method of rendering a ferruginous article relatively non-corrodible. In addition to this, iron which is so treated has such a molecular structure as to render it particularly well adapted as a base for special finishes of lacquers, paints or enamel. This is a feature of more than passing importance in the brake drum art, because of the fact that the exterior surface of the drum is, in most cases, colored with a suitable paint so as to harmonize with the color scheme of the car. Another advantage resides in the fact that the process, which appears essentially to be a precipitation of a reaction salt within the pores of the metal, serves to fill up depressions or perforations and presents a smoother coating, and for this reason is particularly useful as a method of treating cast iron drums. The skin which is formed as a result of this treatment does not, of course, have the abrasion-resisting properties of a harder alloy steel. However, due to the facility and cheapness of the process, it may be economically employed not only on new drums but on those which have been subjected to rather extended use.

As pointed out hereinbefore, the treatment may be applied to any desired section of the drum. In the drawings, there is shown a brake drum the inner surface of which comprises a skin or ring molecularly bonded to the ferruginous foundation metal. This is particularly useful in a brake drum which is constructed for use with an internal band brake. However, it will be appreciated that both the interior and exterior surfaces of the braking flange may be coated, or if desired, the en-

tire drum may be provided with the protective coating.

While there has been described a particular treatment, it is to be understood that this is subject to wide modification and it is to be understood that the invention is not limited to any particular type of treatment. The invention is conceived to reside in the protection of a brake drum which comprises molecularly bonded metals and/or metallic compounds which impart the desired characteristic of lowered corrodibility.

I claim:

1. A parkerized brake drum.
2. A brake drum comprising a ferruginous foundation metal and a surface including a phosphatic salt of the foundation metal.
3. A brake drum comprising a ferruginous foundation metal and a molecularly bonded surface of an inorganic salt of the foundation metal.
4. A brake drum comprising a ferruginous foundation metal and an integral surface comprising a substance containing phosphorus.
5. A brake drum comprising a ferruginous foundation metal and a molecularly bonded inorganic salt of the foundation metal having a lower corrodibility than the foundation metal.
6. A brake drum comprising a ferruginous foundation metal and a phosphatic salt molecularly bonded thereto.
7. A brake drum having a parkerized braking flange.
8. A brake drum having a parkerized exterior surface.
9. A brake drum having a parkerized frictional surface.
10. A brake drum comprising a ferruginous foundation metal and a surface thereon in which a phosphate is molecularly incorporated.

In testimony whereof I affix my signature.

RAYMOND J. NORTON. 110